

Jan. 8, 1963

A. R. A. BEEBER ETAL

3,072,482

SUBBED PHOTOGRAPHICALLY SENSITIVE FILM ELEMENT

Filed Jan. 10, 1958



INVENTOR.  
ALLAN R. A. BEEBER  
BY JAROMIR KOSAR

*J. Russell Jeter*  
ATTORNEY

## 1

3,072,482

SUBBED PHOTOGRAPHICALLY SENSITIVE  
FILM ELEMENT

Allan R. A. Beeber, Elizabeth, N.J., and Jaromir Kosar, Beechhurst, N.Y., assignors to Keuffel & Esser Company, Hoboken, N.J., a corporation of New Jersey

Filed Jan. 10, 1958, Ser. No. 708,278

10 Claims. (Cl. 96—75)

This invention relates to subbing or anchoring layers for use in photosensitive materials. Such layers are used for example in order to anchor a photographic emulsion or the like to a base sheet. More specifically the invention relates to subbing or anchoring layers including methyl vinyl ether-maleic anhydride polymer or its esters.

As is known in the art it is ordinarily necessary in the manufacture of photosensitive materials to make use of subbing or anchoring layers in order to affix a photosensitive layer to a suitable support or base sheet. In the case of ordinary photographic film for example, the support is usually prepared from a cellulose derivative such as cellulose nitrate, cellulose acetate, and other cellulose esters such as cellulose propionate, cellulose butyrate, cellulose acetate-propionate, cellulose acetate-butyrate and the like. Ethers of cellulose, such as methyl ether, ethyl ether and the like are also used. Other types of films such as polyethylene terephthalate film which may be orientated or unorientated are also used in the preparation of photosensitive materials. Woven glass fabrics impregnated with a polyester resin or polystyrene have also been used. In addition, tracing cloth, transperentized papers such as tracing paper and ordinary paper are used as base materials for photosensitive coatings. All of these base materials other than ordinary paper are hydrophobic.

The manner of securing the proper adhesion of photosensitive layers to the various types of hydrophobic base materials constitutes a serious problem. However, the problem is not one of simple adhesion since many compounds known as adhesives are not satisfactory for producing anchorage. The degree of adhesion of the layers to the base must be neither too great, in which case the resulting film is brittle, nor too slight, in which case the layers of the film strip or peel from the support. In most cases the support is hydrophobic and when some hydrophilic substance, such as gelatin is coated onto a hydrophobic base, it is found that there is little or no adhesion between the two. As a matter of fact, a hydrophilic layer can be peeled from such a support with complete ease.

Thus, in the preparation of photosensitive materials, it is very often necessary to permanently affix a water-permeable colloid layer to a hydrophobic support. In order to secure adequate adhesion between the photosensitive layer and the support, it is necessary to impart a hydrophilic nature to the surface of the base sheet. This is accomplished by treating the base sheet with what is known as a "subbing solution." Ordinarily, the subbing material should be soluble or dispersible in a solvent which will dissolve or soften the surface to be coated. This will help to anchor the subbing material to the surface of the base sheet. The subbing material should also form a coating free from tackiness so that the subbed material can be rolled and stored prior to the application of further coatings. The subbing layer should be resistant to stripping when dry or when soaked in water. The subbing layer should be water-permeable, free from color and transparent and it should not desensitize or artificially age the photosensitive layer.

In the past, hydrophobic base materials for photosensitive layers have been coated with gelatin dispersions in organic solvents such as ethyl alcohol, acetone, ethyl

## 2

acetate and mixtures of these solvents. However, in many cases the adherence was not satisfactory and the top-layer could be flaked off by flexing the base sheet.

Now it has been found that the addition of vinyl methyl ether-maleic anhydride polymer or its esters to the coating system improves the anchoring properties considerably. For example a hydrophobic base sheet can be coated with a solution of vinyl methyl ether-maleic anhydride polymer and then after this treatment, the base material is coated with a conventional gelatin subbing solution and finally with a photographic emulsion. For this purpose the vinyl methyl ether-maleic anhydride polymer may be dissolved in alcohols, ketones, acetates or mixtures of these solvents. The solution should contain at least 0.1 percent and no more than 10 percent of the vinyl methyl ether-maleic anhydride polymer or its esters.

Another way of practicing the invention is to coat the base sheet with a synthetic resin solution containing at least 0.01 percent and no more than 10 percent of vinyl methyl ether-maleic anhydride polymer or its esters, following this with a gelatin subbing and a photographic emulsion. The synthetic resin may for example be a cellulose ester, an alkyd resin or the like.

25 A third way is to coat the base sheet with a gelatin subbing solution including no less than 0.01 percent and no more than 5 percent of vinyl methyl ether-maleic anhydride polymer or its esters, coating the usual photographic emulsion upon the base sheet subbed in this manner.

Vinyl methyl ether-maleic anhydride polymer is commonly referred to as PVM/MA.

The application of the various layers to the base sheet may be carried out in any known manner. The base material is coated with one of the solutions described and after this coating has dried, it is followed by the next layer to be used. The sensitive emulsion layer is finally coated over the subbing layers.

40 The objects of the invention discussed above and the means for their attainment will be better understood after reading the following description taken in connection with the accompanying drawing in which:

FIG. I is a view in enlarged diagrammatic section of the photosensitive material described in Example I.

45 FIG. II is a view in enlarged diagrammatic section of the photosensitive material described in Example II.

FIG. III is a view in enlarged diagrammatic section of the photosensitive material described in Example III.

50 FIG. IV is a view in enlarged diagrammatic section of the photosensitive material described in Example IV.

FIG. V is a view in enlarged diagrammatic section of the photosensitive material described in Example V.

55 FIG. VI is a view in enlarged diagrammatic section of the photosensitive material described in Example VI.

*Example I*

As illustrated in FIG. I the base material of cellulose acetate is coated with 2% solution of polyvinyl methyl ether-maleic anhydride in a mixture of ethyl alcohol and acetone. The resulting layer 3 is dried for about two minutes at about 150° F. The polymer layer is then coated with a gelatin subbing layer 2 consisting of a 1% gelatin solution in a mixture of 50% ethyl alcohol and 50% acetone. A silver halide emulsion layer 1 is coated on this gelatin subbing layer. The photosensitive material produced in this manner exhibits excellent adhesion between the photosensitive layer and the base material and is free of objectionable brittleness. The subbing layer has no adverse effect upon the photographic gelatin silver-halide emulsion.

## Example II

As shown in FIG. II the base material of tracing cloth 24 is coated with a nitrocellulose lacquer 25 which serves as a waterproofing layer to prevent moisture from affecting the starch used to transparentize the cloth. This, in turn, is coated with a 3% solution of the butyl ester of polyvinyl methyl ether-maleic anhydride in butyl alcohol. The resulting layer 23 is then coated with a subbing solution of the following composition:

|                | Parts |
|----------------|-------|
| Gelatin        | 1.0   |
| Water          | 5.0   |
| Salicylic acid | 0.8   |
| Methyl alcohol | 75.0  |
| Acetone        | 225.0 |

This forms the layer 22. A bichromated colloid layer 21 including a silver halide is coated on this subbing layer. The anchorage of the colloid layer to the base material in this photosensitive material is excellent when the material is wet or dry. The subbing layers have no adverse effect upon the photosensitive layer. As is known in the art, this type of photosensitive layer is developed after exposure to ultraviolet light by washing off the unexposed areas and blackening the remaining image areas with a conventional silver halide developer.

This type of bichromated colloid photosensitive layer may be applied over some of the combinations of layers disclosed in the other examples and figures of the drawing. However, this type of layer does not coat well directly on a layer which contains PVM/MA. It may be coated readily over a conventional gelatin subbing layer which has been applied over other layers which may include PVM/MA.

## Example III

As shown in FIG. III a polyethylene terephthalate film 34 is coated with a mixture of cellulose nitrate and the butyl ester of vinyl methyl ether-maleic anhydride copolymer of the following composition:

|                       |        |
|-----------------------|--------|
| Nitrocellulose        | 14.0   |
| Ethyl alcohol         | 1400.0 |
| Cellosolve            | 45.0   |
| 5% PVM/MA-butyl ester | 98.0   |

This forms the subbing layer 36. After drying for about 2 minutes at about 200° F. this layer is coated with a gelatin subbing solution consisting of 1% gelatin and a mixture of 30% ethyl alcohol and 70% acetone to form the gelatin subbing layer 32. A silver halide emulsion 31 is coated thereon. The superposed layers have good adherence to each other. No evidence of any tendency for the layers to separate after treatment in various photographic processing baths was noted.

## Example IV

As shown in FIG. IV the base material 44 consisting of glass fabric impregnated with a polyester resin is coated with a discrete layer of alkyd resin 48 and subbed with a gelatin solution of the following composition:

|                                       | Percent |
|---------------------------------------|---------|
| Gelatin                               | 1       |
| Water                                 | 2       |
| Acetic acid                           | 10      |
| Ethyl alcohol                         | 45      |
| 10% solution of butyl ester of PVM/MA | 5       |
| Acetone                               | 37      |

This forms the subbing layer 47. A gelatin silver halide emulsion is coated directly onto the subbing layer 47 and the resulting emulsion layer 41 is dried. The emulsion layer has excellent wet and dry adherence to the base material by virtue of the anchoring substratum. The substratum does not cause any desensitization or artificial aging of the gelatin silver halide emulsion.

## Example V

As shown in FIG. 5 the base material consisting of transparentized paper 54 is subbed with a conventional gelatin subbing solution 52 as described in Example III. The material is then coated with a 5% solution of polyvinyl methyl ether-maleic anhydride in methyl alcohol to form a layer 53. After drying for about 1 minute at 180° F., a cellulose acetate layer is coated thereon. This layer is saponified by a caustic solution and sensitized with a diazotype solution of the following composition:

|                       | Grams |
|-----------------------|-------|
| Diazo diethyl aniline | 50    |
| Citric acid           | 60    |
| Boric acid            | 20    |
| Resorcinol            | 25    |
| Thiourea              | 20    |
| ZnCl <sub>2</sub>     | 10    |
| Water, up to 4000 cc. |       |

The upper three layers of this example may also be applied over a glass fabric base impregnated with a polyester resin which has been coated with an alkyd resin or over a polyethylene terephthalate base sheet which has been coated with a layer containing a cellulose ester and PVM/MA.

## Example VI

As shown in FIG. VI a polyethylene terephthalate film 64 is coated with a mixture of cellulose nitrate and the butyl ester of vinyl methyl ether-maleic anhydride copolymer. This subbing layer 63 is then coated with a brownprint sensitizing emulsion of the following composition:

|                                          | Grams |
|------------------------------------------|-------|
| Ferric ammonium oxalate                  | 10.0  |
| Ferric oxalate                           | 11.0  |
| Silver nitrate                           | 2.5   |
| Water                                    | 120.0 |
| Tartaric acid                            | 3.0   |
| Rhoplex WN 75 (acrylic resin dispersion) | 80.0  |
| Elvacet (polyvinyl acetate dispersion)   | 50.0  |

This forms the light sensitive layer 62. The ferric salts and tartaric acid are dissolved in water and a solution of silver nitrate is added very slowly under constant stirring. Then the Rhoplex WN 75 and Elvacet are added.

The anchorage of the sensitizing layer to the support is excellent whether the material is wet or dry.

Various solvents may be used in the gelatin subbing compositions and these solvents may be chosen according to their action on the base material. For example, when a cellulose acetate base is used a low molecular weight alcohol or a ketone or a mixture of alcohol and ketone may be employed. The ratio of alcohol to ketone ranges from about 50-50% to 75-25%, respectively. When the base material is cellulose acetate-propionate film, an alkyd ester, such as, for example methyl acetate, ethyl acetate, butyl acetate and the like may be effectively employed. In general a wide variety of organic solvents or solvent mixtures may be used for the various base materials so long as the solvent wets or attacks the surface of the base material, i.e. the base is somewhat soluble in an organic solvent or organic solvent mixture. Since the materials suitable for base materials and their solvent properties are known, a person skilled in the art would have no difficulty in selecting a suitable solvent or solvent combination for use in the subbing composition.

As shown by the examples, the subbings including polyvinyl methyl ether-maleic anhydride or its esters are not necessarily used alone but may if desired be used in conjunction with conventional subbing layers such as gelatin, water-sensitive cellulose esters, water-proofing layers and filter layers. It is also possible to incorporate anti-halation dyes in some of these layers.

As shown in the examples, the invention is not limited to silver halide as the light sensitive material since other types of light sensitive materials may also be used. For example, the light sensitive material may be a bichromated hydrophilic colloid such as, gelatin, glue, gum arabic or polyvinyl alcohol sensitized with potassium bichromate or a diazido compound. These layers may or may not also include a silver halide salt as a pigment. Light sensitive ferric salts as used in blueprint paper or in brownprint paper in combination with silver salts other than halides may also be used as the light sensitive material. Diazo compounds with or without a coupling component may also be used. When the diazo compounds are used, the sensitivity of the binding or subbing layer to water may be less critical. For example in this case polyvinyl acetate or a cellulose acetate may be used as the binder. The light sensitive layer may also consist of a polymerizable vinyl compound and a photo-reducible dye as described in the article by Gerald Oster in *Photographic Engineering*, vol. 4, No. 3, pages 173-178 (1953).

Having thus described the invention, what is claimed is:

1. A photosensitive material comprising a thin layer having as an essential component at least one component from the group consisting of polyvinyl methyl ether-maleic anhydride and its esters, an organic solvent soluble hydrophobic layer in direct bonded adherent contact with one side of said thin layer, a gelatin layer in direct bonded contact with the other side of said thin layer and a photosensitive component carried by one of the outermost layers of said photosensitive material.
2. The photosensitive material according to claim 1 in which the hydrophobic layer is cellulose acetate providing a base in bonded contact with said thin layer.
3. The photosensitive material according to claim 1 in which the hydrophobic layer is cellulose nitrate and the hydrophobic layer is coated on a base of tracing cloth.

4. The photosensitive material according to claim 1 in which the hydrophobic layer is a cellulose ester and the hydrophobic layer is coated on a base of polyethylene terephthalate.
5. The photosensitive material according to claim 1 in which the hydrophobic layer is an alkyd resin and is coated on a base of glass fabric impregnated with a polyester resin.
6. The photosensitive material according to claim 1 in which the gelatin layer is coated on a base of transparentized paper.
7. The photosensitive material according to claim 1 in which the gelatin layer is in direct bonded contact with transparentized paper base, and said hydrophobic layer is cellulose acetate, said cellulose acetate having its outer surface saponified and said photosensitive component being a diazo compound incorporated in said outer saponified surface of said cellulose acetate.
8. The photosensitive material according to claim 1 in which the thin layer includes gelatin.
9. The photosensitive material according to claim 1 in which the hydrophobic material is a cellulose ester and the cellulose ester hydrophobic layer is in bonded contact with a base.
10. The photosensitive material according to claim 1 in which the thin layer includes a cellulose ester.

#### References Cited in the file of this patent

##### UNITED STATES PATENTS

|    |           |                  |       |               |
|----|-----------|------------------|-------|---------------|
| 30 | 2,156,069 | Schlack          | ----- | Apr. 25, 1939 |
|    | 2,204,608 | McNally et al.   | ----- | June 18, 1940 |
|    | 2,282,890 | Schneider et al. | ----- | May 12, 1942  |
|    | 2,334,215 | Nadeau et al.    | ----- | Nov. 16, 1943 |
| 35 | 2,699,392 | Herrick et al.   | ----- | Jan. 11, 1955 |
|    | 2,794,742 | Fowler et al.    | ----- | June 4, 1957  |
|    | 2,848,327 | Eichorn          | ----- | Aug. 14, 1958 |